

July 21, 1953

H. TANCZYN

2,646,352

ALLOY STEEL PRODUCTS

Filed April 8, 1947.



Inventor

HARRY TANCZYN

*John Edward Jayant*  
His Attorney

## UNITED STATES PATENT OFFICE

2,646,352

## ALLOY STEEL PRODUCTS

Harry Tanczyn, Baltimore, Md., assignor to  
Armco Steel Corporation, a corporation of Ohio

Application April 8, 1947, Serial No. 740,120

3 Claims. (Cl. 75—126)

1

This invention relates to stainless steel and more especially to manufactures produced from the steel.

Among the objects of my invention is the provision, with savings in material, of stainless steels which are substantially free of detrimental inclusions that ordinarily impair the general surface appearance, and which steels are amenable to working and fabricating into a host of corrosion-resistant products all having substantial freedom from surface imperfections such as black spots, blisters, pits and inclusion lines.

Other objects in part will be obvious and in part pointed out hereinafter.

The invention accordingly consists in the combination of elements, composition of ingredients and mixture of materials, and in the articles, products and manufactures thereof, as described herein, the scope of the application of which is indicated in the following claims.

In the single figure of the accompanying drawing is a diagram showing curves for certain specific values of chromium in my stainless steels and products, and the amounts of manganese and minimum amounts of silicon which are useful along with the specific chromium contents for the prevention of detrimental silicate inclusions.

As conducive to a clearer understanding of certain features of my invention, it may be noted at this point that stainless steel is recognized as being carbon steel which contains about 10% to 35% chromium, with or without nickel (the nickel in so-called straight chromium grades of the steel being even so high as about 3% or entirely omitted) and with or without supplemental amounts of such elements as cobalt, copper, molybdenum, tungsten, vanadium, columbium, titanium, selenium, sulphur, phosphorus, or the like, for special purposes, and the balance substantially all iron.

The art of producing stainless steel has grown during the years from the plain carbon steel industry, and in the course of development from this basic industry, a number of practices and beliefs associated with the carbon steel techniques of manufacture were transmitted to the new craft. Many of these practices were sound; others though rigidly adhered to, lacked proper metallurgical basis when applied to stainless steel, despite being valid for plain carbon steels. It follows then that the most reliable approach to the solution of problems in the stainless steel art, involves thinking in terms of the related highly specialized field.

In connection with the above, it is interesting to observe that for many years, the use of manganese in certain quantities in plain carbon steels has been accepted as imperative for securing desired properties, as for example amounts

2

between about 0.3% and 0.5% for the prevention of hot shortness in rolling and forging operations. The common explanation of the value of manganese in the elimination of hot shortness in ordinary carbon steels is that this element combines with sulphur, thereby forming manganese sulphides. Where manganese is not present in appreciable quantities, other sulphides, namely iron sulphides, having a relatively low melting point are formed, these becoming liquid or semi-liquid at rolling temperatures and accordingly impairing the hot rolling properties.

Manganese also is of benefit in preventing hot shortness, in plain carbon steels because it forms a solid solution with iron oxide. This oxide is dispersed freely through plain carbon steels, and its effect is deleterious in hot working operations unless controlled by such elements as manganese. The solid solution promoted by manganese has a higher melting point than pure ferrous oxide; thus the melting of low temperature constituents is avoided and hot shortness prevented. Among other functions of manganese in the plain carbon steels is that of promoting deep-hardening properties if used in amounts around 1%. Still greater quantities of this element tend to increase wear resistance.

The practice of using manganese in the plain carbon steels, for the purposes described, has carried over the manufacture of stainless steels. In fact, the belief in the importance of manganese in stainless steels has become so entrenched that buyers of straight chromium steels, for example, require substantial amounts of the element to be present according to specifications, and even the manufacturers of these steels have set up definite manganese requirements. In many instances, however, it seems that no serious investigation has been made as to whether this element is wholly beneficial and desirable.

The straight chromium stainless steels are highly susceptible to the development of black spot defects and similar unsightly blemishes which mar the metal surface, these spots often being observed on the surface of sheet, strip, wire or other products following such operations as rolling and polishing. Upon being deformed at working temperatures, the steels take on extended or elongated dark areas of sometimes vastly increased size which may amount to as much as one square inch or more in surface area. In the stainless cutlery steels these black spots often disrupt the finish of such polished products as knives, spoons and the like by constituting a series of streaks, pits and lines which are difficult if not impossible to remove by further polishing.

In hot rolled stainless steel strip and sheet, difficulty also is encountered with "blisters" which are caused by imbedded masses of inclu-

sions; these "blisters" are unsightly and destroy the usefulness of the metal on which they occur. A further difficulty encountered with many of the straight chromium grade stainless steels is the tendency of the alloy metal toward pitting to an objectionable extent when exposed to passivation treatment in such acids as nitric acid. Under these conditions, the metal suffers flash attack, during which an evolution of gas occurs for a few seconds before achieving passivation. This attack, while not long in duration, frequently causes rough surfaces and hurtfully affects the appearance of the finished stainless steel or even, in severe cases, renders the steel useless for certain purposes, particularly for uses where reasonably smooth finishes are of importance.

An outstanding object of my invention accordingly is the provision of wrought and passivated straight chromium stainless steel articles and products, as for example, wire, sheet, strip, or the like, which whether in the polished or unpolished condition are substantially without detrimental silicate inclusions of the character indicated and are substantially free of attack from passivation.

I find that the poor surface condition of straight chromium stainless steels is traceable to the character of non-metallic inclusions present and their size and frequency of occurrence in the steels. There are in fact several different general classes of non-metallic inclusions in these steels, among which are relatively simple non-complex inclusions such as of silica-type; also, low melting point malleable complex inclusions which usually are much elongated in forming or rolling or other working and are the source of such evils as black spots and similar unsightly blemishes in polished sheets. The larger size complex inclusions upon being deformed at working temperatures, as in rolling the metal, are elongated or extended to produce dark areas and black spots. The simple non-complex silica inclusions usually occur in smaller form, are relatively hard, and do not elongate as readily as the complex ones at hot working temperatures, are much less visible on polished stainless steel articles and products, and are generally not troublesome.

My explorations into the causes of complex silicate inclusions have revealed that manganese promotes the development of these inclusions in the straight chromium steels, depending upon the amount of chromium and silicon present. Manganese, chromium and iron tend to reduce the free silica of firebrick in runners, protective sleeves and ladle lining to produce ferrous oxide, manganese oxide, chromium oxide and silicon. The silicon is absorbed by the metal while the ferrous oxide, manganese oxide and chromium oxide flux additional quantities of silica to form the undesirable complex silicate inclusions. Since iron and chromium possess very weak reducing powers with regard to silica whereas manganese is very powerful in this respect, the elimination of manganese from stainless steels will forestall the aforementioned reactions with the firebrick and result in the presence of small, widely-scattered silica inclusions.

The complex silicates may be changed to harmless silica by a proper manganese-to-silicon ratio; the simple silica inclusions are small and non-deformable at hot working temperatures and not readily visible to the naked eye. Of still further importance, where the manganese content is extremely low or substantially absent, the

chromium in these steels in many respects tends to function as a substitute for manganese, such as in producing sulphides, deep-hardening effects where the steels are hardenable, resistance to abrasion, and freedom from hot shortness.

Referring now more particularly to the practice of my invention, I provide 10% to 35% straight chromium stainless steels and products of the steels (as for example wire, sheet, strip, and the like, in the wrought and unpolished or polished condition) in which manganese and silicon are consistent with amounts indicated beneath the appropriate curve in the accompanying diagram, the curve corresponding to the specific amount of chromium used. The chromium curves define highly critical upper limits on the maximum permissible quantity of manganese in the steel, for any specific silicon and chromium contents in achieving simple silica inclusions as distinguished from complex silicate inclusions. Other chromium curves and upper limits on manganese in my steels, of course, may be arrived at in the diagram by interpolation. The steels are of hardening or non-hardening quality, as desired, depending upon the specific composition and its response to heat treatment.

Among the steels and products which I provide are those including about 10% to 35% chromium, up to about 1.5% carbon, manganese below about 0.2%, and silicon from incidental amounts up to 1% or more, the manganese also being consistent with amounts in the accompanying diagram falling beneath the appropriate chromium curve, the remainder of the composition being substantially all iron. In the latter group are steels containing over 0.15% carbon and 12% to 14% chromium, and those containing 0.60% to 1.20% carbon and 14% to 18% chromium as in the form of cutlery products and surgical instruments, respectively. Along with chromium, manganese and silicon, my steels sometimes include nickel up to about 3% and/or quantities of some other element or elements such as molybdenum, zirconium, titanium, vanadium, columbium, sulphur, phosphorus, or selenium, for special purposes. At times the manganese content is zero as where practical considerations in production allow. Quite often, my steels and products are made to have a very low manganese content ranging up to about 0.1%, this content further being in keeping with the low side of the specific chromium curve in the accompanying diagram and not exceeding the maximum amount permitted by the specific silicon content according to the diagram.

I find that not only is an important saving in material effected in my stainless steels and products, where the manganese content is quite low or virtually eliminated, but valuable improvements, in certain properties are had, among these being improved resistance to corrosion and impact, and the substantial freedom from silicate inclusions which ordinarily cause elongated black spots and the like in wrought corrosion-resistant steels.

As illustrative of the practice of my invention, in the production of a straight chromium stainless steel from available and inexpensive raw materials, I prepare a bath of ferrous metal in a suitable furnace, for example, an electric arc furnace, using in the charge such materials as rustless iron scrap and/or ordinary, low-carbon steel scrap, and an oxidizing agent such as iron ore, roll scale or the like. The scrap materials entering the charge are for example of 0.30% to

0.60% manganese grade for simplifying the elimination of manganese during the process to the amount desired in my stainless steels. Any other substantial sources of manganese also are avoided in the furnace. The bath of ferrous metal resulting from the charge has an oxidizing slag or covering which forms during the melting operation. I bring the bath to a uniformly high temperature. Chromium additions are made either along with the initial melt down ingredients, using, for example, high carbon ferrochrome or chrome ore, or these additions may be made to the bath and slag formed as indicated above, as through the use of chrome ore.

Under the action of the strongly oxidizing slag and the high temperatures employed, carbon coming from the furnace electrodes and furnace atmosphere, as well as from the raw materials, is effectively excluded and/or removed from the bath of ferrous metal. A portion of the manganese in the charge passes to the slag and is not fully reduced to metal again. The use of oxidizing agents such as supplemental amounts of the iron ore or roll scale, furthers the elimination of manganese to the slag. Along with the oxidation of carbon and manganese there is an incidental oxidation of chromium from the metal; the chromium oxides formed pass into the slag. After complete melt-down of the various ingredients and at the end of the oxidizing heat the ferrous metal bath has a low carbon content, and a manganese content preferably considerably less than the 0.2% maximum value desired in my stainless steels. The oxide slag covering the bath contains the oxides of iron, chromium and manganese.

I often employ a suitable reducing agent, such as ferrosilicon for recovering iron and chromium from the oxidizing slag. To enable control over silicon contents of the bath, I usually introduce basic slag-forming materials, such as burnt lime, in amounts sufficient to assure basic conditions during the reduction of the oxides in the slag. The basic slag prevents silicon contamination of the bath and allows for adjustment of the silicon contents after the reducing period should adjustment be needed over and above the incidental amounts present.

Under the reducing conditions only a partial recovery of manganese is had, which element passes back to the bath along with the iron and chromium recovered. By careful control over manganese contents of the bath as derived from the furnace charge and the like, however, the recovery of manganese from the slag is not excessive and the manganese content of the bath remains at say for example some value below 0.1%. I draw off the slag and substitute a suitable finishing slag on the surface of the steel. After this, I adjust the contents of the bath to the desired 60 alloy contents as by the addition of low-carbon

ferrochrome, and silicon at least in amounts called for in the accompanying diagram by the specific amounts of chromium and manganese for ensuring the substantial absence of complex silicates in the steel. Other elements as for special purposes are added if desired. I then teem the melt into ingot molds and thus form ingots of the straight chromium steel.

The steels which I provide, whether produced in the electric arc furnace or in any other suitable manner, and whether of ferritic non-hardening quality or of martensitic hardening quality, suffer no appreciable detriment to hot working properties, ultimate tensile strength, yield strength, reduction in area, elongation, machinability, and the like, which might be traced to the control over manganese and silicon in relation to chromium.

For illustrating certain properties of my low-manganese hardening steels, as compared with those of several steels containing an excessive amount of manganese for the silicon and chromium present, refer to specific compositions noted in Table I. It will be seen that Steel A in this table contains a quite small quantity of manganese as permitted by the accompanying diagram. The Steel B, however, has a relatively high manganese content in view of the silicon and chromium contents and is objectionably susceptible to the formation of complex silicates as would be expected in view of the diagram.

Table I.—Hardening steels

| Steel  | C     | Cr    | Mn   | Si   | Ni   | P     | S     |
|--------|-------|-------|------|------|------|-------|-------|
| A----- | 0.097 | 12.13 | 0.06 | 0.26 | 0.06 | 0.013 | 0.013 |
| B----- | 0.096 | 12.20 | 0.52 | 0.29 | 0.02 | 0.006 | 0.012 |

<sup>1</sup> Prior art.

It is to be observed in Table II that many of the beneficial properties of the Steels A and B remain substantially unchanged despite the differences in manganese contents, and the relation of the latter to silicon and chromium. The hardening characteristics of these steels are not materially altered whether the materials are air-cooled or oil quenched from the hardening temperature, such as by heating at 1750° F. for one-half hour, following with an oil quenched and tempering, or by heating at 1150° F. for four hours, thereafter cooling in air and tempering (see Table II). A very surprising feature, however, notable in the table, is that the Steel A, has a higher impact value than the Steel B where both steels are in the hardened and tempered condition. This improved impact resistance is attributed to the manganese content with relation to the silicon and chromium and is a general characteristic of my hardened and tempered steels.

Table II.—Mechanical properties of steels in Table I

| Steel  | Heat Treatment                              | Ult. Tens. Str., p.s.i. | 0.2% Yld. Str., p.s.i. | Elong. Percent, 2" | Red. of Area, Percent | Izod Impact | Brinell Hard-ness |
|--------|---------------------------------------------|-------------------------|------------------------|--------------------|-----------------------|-------------|-------------------|
| A----- | 1,150° F. (4 hrs.) air Cooled and Tempered. | 115,700                 | 98,350                 | 20.0               | 68.7                  | 99          | 251               |
| B----- | 1,150° F. (4 hrs.) air Cooled and Tempered. | 113,500                 | 99,000                 | 20.0               | 68.9                  | 85-86.5     | 248               |

The non-hardening stainless steels which I provide, also have improved impact resistance by reason of the proper manganese content in relation to silicon and chromium, or because of the virtual elimination of manganese. One of my non-hardenable ferritic stainless steel compositions is represented by Steel C in Table III; the Steel D noted for comparison, has a manganese-to-silicon and chromium relation outside the desired limits.

Table III.—Non-hardening steels

| Steel  | C    | Cr    | Mn   | Si   | Ni   | P     | S     |
|--------|------|-------|------|------|------|-------|-------|
| C..... | .068 | 16.60 | 0.09 | 0.35 | 0.20 | 0.014 | 0.012 |
| D..... | .060 | 16.56 | 0.44 | 0.41 | 0.21 | 0.016 | 0.012 |

<sup>1</sup> Prior art.

It will be seen in Table IV, that after like heat treatment, the non-hardening Steel C has superior impact resistance as compared with the excessively high-manganese Steel D which also is of non-hardening quality.

Table IV.—Mechanical properties of steels in Table III

| Steel  | Annealing Treatment                               | Ult. Tens. Str., p. s. i. | 0.2% Yld. Str., p. s. i. | Percent Red. area | Percent Elong. in $\frac{1}{2}^{\prime\prime}$ | Izod Impact | Brinell Hardness |
|--------|---------------------------------------------------|---------------------------|--------------------------|-------------------|------------------------------------------------|-------------|------------------|
| C..... | 1,450° F. to 1,475° F. (4 hrs.) and water quench. | 69,500                    | 37,650                   | 72.0              | 37.5                                           | 37-50       | B-78             |
| D..... | 1,450° F. to 1,475° F. (4 hrs.) and water quench. | 66,900                    | 37,600                   | 68.9              | 35.5                                           | 14-9        | B-82             |

My stainless steels, whether hardening or non-hardening are highly resistant to corrosion in various acids such as nitric, acetic, sulphuric or hydrochloric acid, and under a wide variety of other conditions, as for example those involving corrosive gases, heat, moisture or the like. A further valuable asset of my stainless steels is that they display outstanding resistance to flash attack as when immersed for passivation in a nitric acid solution. Where desired, therefore, I subject the steels to passivation treatment, and with highly satisfactory results. The treated metal is substantially free of pits, blemishes, and other results of flash attack.

My straight chromium steels are successfully worked, formed and fabricated and by such operations as forging, rolling, drawing, stamping, machining, welding, or any other of a host of permissible operations, I provide products of the steels. These products by reason of the substantial freedom of the metal from complex silicate inclusions take on a highly satisfactory surface finish such as where the surface is polished or finished without a polish. I sometimes subject my steel products to an electrolytic polishing treatment, as of any conventional type used in the polishing of stainless steels. The polished surface is substantially free of blisters, black spots and hair-line defects which so frequently occur from inclusions in excessively high-manganese, straight chromium stainless steels.

Apart from such products as wire, sheet, strip, and the like which I make from my stainless steels, the metal is fabricated when desired into a host of other products, among these being valve parts including stems, shafts, valve balls, valve trim, seats or rocker arms. A further category of my products includes carburetor parts which handle corrosive gasolines. In precision instru-

ments, my stainless steels are often made to function as needles, spring, fittings, gimbals and indicators. I also make cutlery including such products as scissors, knives, ice picks, and other culinary items. On other occasions the steels are fabricated into dairy equipment, trim and hardware for house, office or restaurant use, or into chemical plant equipment, particularly for nitric acid plants and illustratively including pipes, towers, tanks, heat exchangers and the like. Still other products of the steel fall into a miscellaneous group comprising such articles as propellers for motor boats and outboard engines used in salt water, solenoid magnet cores, pneumatic tools where exposure to weather and shock are encountered, turbine blades, seaming rolls for can-filling machinery, surgical instruments, dental instruments, and a variety of tools such as wrenches, screw drivers and saws as where toughness and corrosion resistance are desirable. While many further products of my stainless steels could be specifically identified, it is believed that the above will suffice for purposes of illustration.

Thus it will be seen that in this invention there are provided straight chromium stainless steels and products in which the various objects hereinbefore set forth together with many thoroughly practical advantages are successfully achieved. It will be seen that the alloys are hardening or non-hardening by heat treatment, depending upon specific composition and the manner of heat treatment, and the products and the steels themselves are substantially free of black spots. It will also be appreciated that the steels are workable and capable of being finished by polishing and passivation treatment with highly satisfactory results and are well suited for resisting corrosion in use.

While considerable emphasis has been placed upon the accompanying diagram and the relation of manganese, silicon and chromium there prescribed, it will be appreciated that the chromium to some extent may be replaced by partial substitution in actual practice within the scope of the invention.

As many possible embodiments may be made of my invention and as many changes may be made in the embodiment hereinbefore set forth, it will be understood that all matter described herein is to be interpreted as illustrative and not as a limitation.

I claim:

1. In manufactures of the class described, wrought and polished straight chromium stainless steel sheet, strip, wire, and like products containing large amounts of chromium and small amounts of manganese and silicon which products are substantially free of surface-defacing complex silicate inclusions and comprise 10% to 27% chromium, up to about 0.2% manganese and from incidental amounts up to about 1% silicon with said manganese content restricted

to amounts beneath the curve in the accompanying diagram corresponding to the specific amount of said chromium, and the remainder substantially all iron.

2. In manufactures of the class described, wrought and polished straight chromium stainless steel products containing substantial amounts of chromium and small amounts of manganese and silicon which products are substantially free of surface-defacing complex silicate inclusions and comprise at least 0.15% carbon, 12% to 14% chromium, less than 0.2% manganese and from incidental amounts up to 1% silicon with said manganese and silicon contents falling beneath the curve in the accompanying diagram corresponding to the specific amount of said chromium, and the remainder substantially all iron.

3. In manufactures of the class described, wrought and polished straight chromium stainless steel products containing substantial amounts of chromium and small amounts of manganese and silicon which products are substantially free of surface-defacing complex silicate inclusions and comprise 0.60% to 1.20% carbon, 16% to 18% chromium, less than 0.2% manganese and from incidental amounts up to 1% silicon with said silicon and manganese contents falling beneath the curve in the accom-

panying diagram corresponding to the specific amount of said chromium, and the remainder substantially all iron.

HARRY TANCZYN.

References Cited in the file of this patent

UNITED STATES PATENTS

| Number    | Name          | Date          |
|-----------|---------------|---------------|
| 1,893,004 | Shimer et al. | Jan. 3, 1933  |
| 1,924,043 | Kinzel        | Aug. 22, 1933 |
| 2,087,431 | Feild         | July 20, 1937 |

FOREIGN PATENTS

| Number  | Country       | Date          |
|---------|---------------|---------------|
| 315,444 | Great Britain | July 15, 1929 |

OTHER REFERENCES

Chemical and Metallurgical Engineering, July, 1927, pages 417, 418, 419.

Stainless Iron and Steel, 2nd edition, pages 103, 107, 109, 129, 141, 218, 306, 416, 439, 467, 496 to 504, 520, 543. Edited by Monypenny. Published in 1931 by Chapman and Hall, London, England.

Book of Stainless Steel, 2nd edition, pages 149 to 156. Edited by Thum. Published in 1935 by the American Society for Metals, Cleveland, Ohio.